

May 18, 1937.

F. E. BARTELL

2,080,905

THREAD ELEMENT AND PROCESS AND APPARATUS FOR MAKING IT

Filed Jan. 20, 1936



## UNITED STATES PATENT OFFICE

2,080,905

THREAD ELEMENT AND PROCESS AND  
APPARATUS FOR MAKING IT

Floyd E. Bartell, Ann Arbor, Mich., assignor to  
G. E. Wilder, William A. Defnet, Sherwood  
Field, J. Hugo Smith, Frank MacKenzie,  
Yellott F. Hardcastle, D. Kenneth Laub, Dun-  
can J. McNabb, and Stanley V. Laub, all of  
Detroit, Mich.

Application January 20, 1936, Serial No. 59,831

6 Claims. (Cl. 117—2)

The invention relates generally to textiles and it has particular relation to a threadlike element and a process and apparatus for manufacturing it. It also constitutes a continuation in part of 5 the subject matter embodied in my co-pending application Serial No. 36,796, filed August 19, 1935.

One object of the invention is to provide an improved thread that can be manufactured in- 10 expensively.

Another object of the invention is to provide an improved thread that is substantially imperforate and which is highly resistant to the passage of water therethrough.

15 Another object of the invention is to provide an improved thread of the above character that may be readily made of different denier.

Another object of the invention is to provide an improved threadlike element, which may be 20 used as a bristle for brushes or the like.

Another object of the invention is to provide a process of manufacturing thread of the above described character that will enable production of a uniform product and also enable production 25 of threads varying in denier.

Another object of the invention is to provide an apparatus for manufacturing thread of the above identified character in a simple and inexpensive manner.

30 Other objects of the invention will become apparent from the following specification, the drawing relating thereto and from the claims hereinafter set forth.

For a better understanding of the invention, 35 reference may be had to the drawing wherein:

Fig. 1 is a vertical and longitudinal cross section of an apparatus employed in manufacturing thread or the like according to one form of the invention;

40 Fig. 2 is a cross sectional view on a larger scale taken substantially along line 2—2 of Fig. 1;

Fig. 3 is a cross sectional view on a larger scale taken substantially along line 3—3 of Fig. 1;

45 Fig. 4 is a cross sectional view on a larger scale taken substantially along line 4—4 of Fig. 3 and illustrating generally the character of the several filaments used in manufacturing the thread; and

Fig. 5 is a fragmentary cross-sectional view 50 illustrating a form of apparatus that may be employed to produce a flattened thread.

According to one form of the invention, a plurality of filaments 10 of cellulosic material such as cellulosic acetate, cellulosic nitrate, or the like, are provided on supply spools 11 rotatably

5 mounted on a pin 12 supported by brackets 13. Each of the filaments, as best shown by Fig. 4, comprises a number of loose minute filaments 14 and it will be understood that the collected minute filaments constitute a commercial thread 10 that is now produced from cellulosic material. The filaments 10 lead through a suitable guide bracket 15 provided with a guide aperture 16 for each individual filament 10, and then the filaments pass through a tank or vat 17 containing 10 a treating solution 18 capable of gelatinizing or softening the cellulosic material, a pivoted drop arm 19 is provided with a guide notch 20 for collecting and keeping the filaments 10 immersed 15 in the solution 18 during their passage through 15 the tank or vat 17.

The treating solution 18 may be termed a gelatinizing agent for cellulose esters, and is composed preferably of ethyl acetate, acetone, or other so-called "solvent" for cellulose esters. 20 While cellulose probably does not form a true solution in any of its ordinary solvents, it may be dispersed colloidally by such solvents. In limited amounts of such solvents, swelling of the esters occurs and a gel is formed. The exact 25 nature of the gel formation is not fully understood, but it is believed that the solid or semi-solid material portion of the gel is converted to the colloid state, in which state it possesses a very great specific surface area; that is, large 30 surface area per unit volume of material; hence a great interfacial energy which effects in a product, high cohesion and high adhesional properties. Ethyl acetate is an excellent, fast evaporating, gelatinizing agent for cellulose acetate. 35 Acetone is likewise a fast evaporating solvent, peptizing or gelatinizing agent for certain cellulose esters, resin and many other organic compounds. A solution of alcohol and ether (as 75% alcohol, 25% ether) is a gelatinizing agent for 40 cellulose nitrate.

The time the filaments are allowed to remain 45 in the solution 18 is of importance. If allowed to remain too long, the cellulosic material comprising the filaments may be dissolved and pass into the solution, in which event the filaments would lose their identity as such. It is desired to retain the filaments in the solution only for a time sufficient to gelatinize and soften the outer surface portion of each minute filament, while leaving a central core thereof substantially unaffected, and ordinarily all minute filaments will be acted upon by the solution owing to the fact that the latter is quite volatile and quickly penetrates in and between filaments. It may be 50 55

that the minute filaments 14 would be grouped closely enough so as to prevent the solution reaching each minute filament at all points, but it seems that all or substantially all of the outer 5 surface of each minute filament 14 can be acted upon by the solution. It is also possible that the action may vary to some extent as the solution will touch the outer minute filaments perhaps an infinitesimal instant before reaching 10 the inner minute filaments. The desirable result is that all minute filaments will have their outer surface portions gelatinized so that subsequently all of the collected filaments may become bonded in an integral mass, but it will be 15 appreciated that some variation might be obtained. For example, if it be assumed that one of the inner minute filaments is not acted upon by the solvent, the outer group of minute filaments still would integrally bond together 20 around the unaffected filament. This is mentioned for the reason that it is difficult to determine that any one inner minute filament or part thereof is unaffected. Experiments seem to indicate the solution quickly penetrates 25 between all minute filaments and gelatinizes the outer surface portion of each.

After leaving the solution, the collected filaments pass through a rotary tube 22 mounted in bearings 23. The tube is provided with a bevel 30 gear 24 that meshes with a gear 25 in turn driven by a shaft 26. The latter at its lower end has three pulleys 27, 28 and 29, the latter pulley being engaged by a belt 30 that is trained about a pulley 31 on the shaft of a motor 32. The right end of 35 the tube has a flared mouth to facilitate passage of the filaments thereinto and to avoid an undesirable scraping action on the filaments, and the left end of the tube has a stopper 33 composed of cork, rubber or other suitable material. The 40 stopper has an axial opening 34 through which the filaments pass and it seems preferable that this opening be slightly eccentric to the axis of the tube, although it may be concentric. It is of such size, however, that rotation of the stopper 45 with the tube causes an appreciable twisting or frictional force to be applied to the outer surface of the grouped filaments passing therethrough so as to compact the filaments closely together, while at the same time cause the outer surface 50 of the group to be rendered smooth, substantially round and imperforate. Moreover, the compacting of the filaments substantially removes any voids between the minute filaments, so as to leave a substantially solid, round, imperforate 55 thread element 35 having a smooth outer surface.

After the filaments leave the solution, with the outer surface portions only of the minute filaments gelatinized, they will become bonded together through surface union of adjacent filaments but the gelatinized condition of the outer surface portions of the minute filaments is retained at least partially until the group enters the stopper so as to permit compacting of the filaments, eliminating voids therein, rounding of the 60 thread and providing a smooth outer surface therefor. Evaporation of the solvent from the filaments begins as soon as they leave the solution, but it is intended that the evaporation will not be sufficient to prevent obtaining the particular results mentioned through action of the rotary stopper and that after leaving the stopper, the form and condition of the thread then may be retained.

It may be mentioned that some twisting of the 75 filaments by the stopper seems to occur between

the stopper and arm 19 and even beyond the latter and accordingly from the time the grouped filaments leave the solution, they are subjected to some forces tending to compact them and to bring them into an integral union as the gelatinized surfaces of the filaments are drawn together. Evaporation of the solvent will continue, of course, but in any event the grouped filaments are still in a formative condition when they pass through the stopper so as to permit some change in the 10 united gelatinized surfaces of the filaments to obtain the desired finished thread condition. It may be added that the apparatus may be so arranged that the filaments do not touch the tube if this is desired. 15

It appears that no permanent twisting of filaments is obtained in the finished thread even though they appear to be in a twisted condition between the stopper and the solution. Possibly there may be some fracturing of filaments, and re-union thereof through the gelatinized material adjacent the fracture, or perhaps there may be a release of the twist after the thread leaves the stopper. In any event, frictional twisting forces are applied, some twisting occurs between the 25 stopper and solution at least, and the finished thread after it leaves the stopper appears substantially to have no twist. 20

The finished thread is wound upon a spool 38 driven through gears 39 and 40, a reduction gear 30 41, a pulley 42 and a belt 43 engaging the pulley and also the pulley 28. The distance between the spool and stopper may be such as to allow complete evaporation of any solvent retained by the thread or a fan 44 for example may 35 be placed adjacent the stopper to accentuate complete evaporation. As shown, the fan is driven by means of a pulley 45 and a belt 46 engaging the latter and the pulley 27. While the results have been satisfactory without a fan, it is reasonable 40 that the fan would act to obtain a quick evaporation of any solvent in the thread as the latter leaves the stopper and it seems desirable to have the solvent evaporate quickly after the thread is 45 finally formed by the stopper. 45

It is to be understood that the tube, stopper and fan are rotated preferably at a high rate of speed while the thread is pulled therethrough by the spool 38 at a relatively slow rate of speed. In this connection it is to be noted that the filaments are 50 under some tension as they move through the stopper and this seems desirable.

It appears that the longitudinal rigidity of the thread is materially increased and this may be caused by hardening and rendering more dense 55 the outer surface portions of the individual filaments. A possible explanation of this result may also reside in the fact that the filaments are stretched through the tension and also the twisting action, resulting in a definite molecular orientation or crystallization of the material with the crystals extending lengthwise of the thread so that the filaments are set in this condition as the treating solution evaporates. The outer portions of the filaments which had been gelatinized 60 or softened, upon drying become relatively hard, 65 firm and flexible.

Various denier threads may be manufactured by increasing the number or size of the filaments 70 10 that are employed. The product may be woven into cloth, curtains and the like, and desirable sizes thereof may be used for bristles in brushes. A great many uses of the product will occur to those interested in this art. The imperforate surface of the product, its solidity and 75

freedom from voids, its water resistant characteristics due to the material and its freedom from voids and perforations, and its integral nature due to integral bonding of the filaments, render 5 it highly useful for manufacturing water resistant fabric, water resistant brushes and the like.

Figure 5 relates to the same apparatus but additionally provides a pair of rollers 48 and 49 10 between which the thread passes after leaving the stopper. It will be understood that the apparatus will be adjusted if necessary to insure that the thread will still be in a formative condition sufficient to permit the rollers to flatten 15 it and then to cause the flattened thread to retain its new form. Various contours of rollers might be used to vary the form of thread obtained in this manner.

As many changes may be made in the above 20 product and many apparently widely different means may be employed for carrying out the method of making the same, it is intended that all matter contained in the above description or shown in the accompanying drawing, shall be 25 interpreted as illustrative and not in a limiting sense.

What I claim is:

1. The method of manufacturing a threadlike 30 element which comprises treating a plurality of filaments of cellulose esters with a gelatinizing solution to soften the filaments, assembling the filaments, applying rotary sliding forces tending to twist the filaments while maintaining them under tension, and then causing evaporation of 35 the solution.

2. The method of manufacturing a threadlike 40 element which comprises passing a plurality of filaments of cellulose esters through a gelatinizing solution to soften and gelate only the outer surface portions of the filaments, assembling the filaments, applying rotary sliding forces tending to twist the filaments, and then causing the solution to evaporate.

3. The method of manufacturing a threadlike 5 element which comprises passing a plurality of filaments of cellulose esters through a gelatinizing solution to soften and gelate only the outer surface portions of the filaments, assembling the filaments and applying rotary sliding forces tending to twist them while maintaining the filaments under tension, and then causing the solution to evaporate.

4. The method of manufacturing a threadlike 10 element which comprises passing a plurality of filaments of cellulose esters through a gelatinizing solution to soften and gelate only the outer surface portions of the filaments, assembling 15 the filaments and applying rotary sliding forces tending to twist them while maintaining them under tension, and then causing the solution to evaporate while maintaining the filaments under tension.

5. The method of manufacturing a threadlike 20 element which comprises passing a plurality of cellulosic filaments through a solvent to gelatinize the outer surface portions of the filaments, bringing the filaments together and applying rotary frictional forces to the assembly to compact the 25 filaments and provide a single element having a smooth, substantially imperforate outer surface and simultaneously bonding the filaments together through union of the gelatinized surface, 30 and then evaporating the solvent.

6. The method of manufacturing a threadlike 35 element which comprises subjecting a plurality of cellulosic filaments to the action of a solvent so as to gelatinize the outer surface portions of the filaments, assembling the filaments and applying 40 rotary frictional forces to the outer surface of the assembly to compact the filaments and provide a single substantially imperforate element having a smooth outer surface and to cause the gelatinized surfaces to unite and bond the filaments together, and then evaporating the solvent.

FLOYD E. BARTELL.